

Nov. 12, 1929.

J. C. FEAGLEY

1,735,383

BOX TOE BLANK

Filed Feb. 4, 1927

Fig. 1



Fig. 2



Fig. 4



Fig. 3



INVENTOR

Joseph C. Feagley  
by his attorneys  
Bynes, Stubbins & Pamplin.

## UNITED STATES PATENT OFFICE

JOSEPH C. FEAGLEY, OF LANCASTER, PENNSYLVANIA, ASSIGNOR TO ARMSTRONG CORK COMPANY, OF LANCASTER, PENNSYLVANIA, A CORPORATION OF PENNSYLVANIA

## BOX-TOE BLANK

Application filed February 4, 1927. Serial No. 165,846.

This invention relates to box toe blanks, and more especially to soft box toe blanks.

During the manufacture of a shoe, the box toe is subject to very severe stretching and pulling. It is placed under the leather which forms the toe proper of the shoe, and it is necessary for a satisfactory product, that the box toe be capable of a considerable amount of stretch in any direction.

10 Box toes have been made of various materials, but a number of them have been unsatisfactory because they have not possessed the ability to stretch the desired amount in various directions. I provide a box toe made of a fibrous backing having a coating thereon, and capable of substantially equal amounts of stretch in all directions. I preferably employ a fabric whose warp threads per unit of width are capable of substantially the same amount of stretch as are the filler threads per unit of width. This may be substantially accomplished by employing a fabric whose warp and filler threads are of substantially the same weight, twist and count.

25 It is desirable that a relatively thin fabric be used. Coarse strand materials, such as burlap, are unsatisfactory because there is a definite limitation upon the total thickness of a box toe. If a heavy fabric, such as burlap, is used, only a thin composition can be applied. This thin composition does not have sufficient strength and peels or rubs away from the heavy fabric when the shoe upper is being "wiped in" around the fore part of the shoe. The "wiping in" operation is a very severe one. The toe cap, lining and box toe materials are worked to a smooth finish around the edge of the last, a pair of curved metal jaws being forced repeatedly across the edge of the last until all of the materials are smoothed down.

35 In the accompanying drawings, which illustrate the present preferred embodiment of my invention:

Figure 1 is a view of a box toe from the fabric side;

Figure 2 is a view from the coating side;

Figure 3 is a perspective view partly broken away showing the skived edge of the box toe; 50 and

Figure 4 is a more or less diagrammatic view, illustrating the fabric employed for the backing.

In making up my improved box toe, I 55 employ a fabric whose warp and filler threads are substantially the same weight and count. In ordinary woven fabrics, the warp threads are of a much harder and finer twist than are the filler threads.

I prefer to use relatively soft twist threads of the character frequently employed for filler threads in both the warp and filler of the fabric. Both the warp and filler yarns are what are known as "8", and have about eight 60 or nine twists to the inch, which is somewhat less than the standard twist. A cotton fabric made to a count of 32 warp and 32 filler threads per inch and weighing approximately 6 ounces per square yard has been found 65 satisfactory. Ordinarily, it is not desirable to use a cloth much heavier than this, because a heavier cloth requires a thinner coating in order to maintain the box toe within the commercial limits of thickness.

70 The fabric is coated with a composition which preferably includes cork as one of its elements. The coating should be such that a soft and non-breakable box toe results. A toe of this character will withstand the operations involved in such manufacture and will be satisfactory in use. It is somewhat moisture absorbent, and therefore, not hot and uncomfortable.

75 Satisfactory mixes for the coating are as 85 follows:

A

2 lbs. crude rubber (smoked sheets)

15 lbs. reclaimed rubber (No. 1 tube reclaimer)

90

4 lbs. hard hydrocarbon (mineral rubber)  
 10 ozs. sulphur  
 2 lbs. zinc oxide  
 5 lbs. earthy filler (china clay)  
 5 40 lbs. ground cork  
 4 ozs. antioxidant

B

350 lbs. oxidized oil and resin cement  
 35 lbs. ochre  
 10 255 lbs. ground cork  
 1/2 lb. lime

The above mixes are desirable, but it will be understood that the quantities of materials used may be varied, or equivalent materials 15 substituted for the various elements.

The box toe is cut from the coated material. As shown in Figure 1, the box toe is so cut that the threads of the fabric backing 2 run diagonally to the box toe. This 20 is particularly desirable with my special fabric as it insures that the box will stretch properly and in substantially equal amounts in any direction.

The fabric is illustrated in Figure 4 as 25 being made of filler threads *f* and warp threads *w* of substantially the same weight and twist, and substantially the same count.

The composition coating 3 extends over the entire box toe, but is skived all around, as 30 indicated at 4 in Figures 2 and 3. It will be noted from Figure 3 that the composition coating is relatively thick, as compared with the fabric. This insures that it will not peel or rub away during the "wiping in" operation. 35

My box toe blanks are softer and therefore much more comfortable than the hard box toe blanks commonly made of leather or fibre or stiffened felt. The resilient character of 40 the cork mix makes the box toe non-wrinkling, as contrasted with the soft upper leather box toes which will wrinkle. Moreover, the tensile structural strength of my box toe is not affected by water or perspiration. The 45 composition herein disclosed is further described and claimed in my copending application for shoe counters, Serial No. 165,845, filed February 4, 1927.

I have illustrated a preferred form of the 50 invention, but it will be understood that it is not limited thereto, as it may be otherwise embodied within the scope of the following claims.

I claim:

55 1. As a new article of manufacture, a soft box toe blank made of extensible fabric whose warp threads per unit of width are capable of substantially the same amount of stretch as are the filler threads per unit of width, the 60 fabric having a coating thereon, the threads of the fabric running diagonally to the box toe.

2. As a new article of manufacture, a soft box toe blank made of extensible fabric whose 65 warp and filler threads are of substantially

the same weight, twist and count, the fabric having a coating thereon, the threads of the fabric running diagonally to the box toe.

3. As a new article of manufacture, a soft box toe blank made of extensible fabric whose warp and filler threads extend diagonally to the longitudinal axis of the toe blank, and a coating on the fabric. 70

4. As a new article of manufacture, a soft box toe blank made of stretchable fabric whose warp and filler threads extend at an angle of substantially 45° to the longitudinal axis of the toe blank, and a coating on the fabric. 75

In testimony whereof I have hereunto set 80 my hand.

JOSEPH C. FEAGLEY.

85

90

95

100

105

110

115

120

125

130